

Aug. 5, 1969

O. G. KOPPIUS

3,459,986

SECONDARY EMISSION CATHODE OR DYNODE OF A POROUS MATRIX OF  
TUNGSTEN OR MOLYBDENUM IMPREGNATED WITH SECONDARY  
EMISSION MATERIAL SUCH AS A TUNGSTATE OR AN  
ALKALI HALIDE OF CALCIUM  
Filed Jan. 27, 1967



STEPS IN FABRICATION OF DYNODE

INVENTOR.

OTTO G. KOPPIUS

BY *Otto G. Koppius*

ATTORNEY

3,459,986

SECONDARY EMISSION CATHODE OR DYNODE  
OF A POROUS MATRIX OF TUNGSTEN OR MO-  
LYBDENUM IMPREGNATED WITH SECONDARY  
EMISSION MATERIAL SUCH AS A TUNGSTATE  
OR AN ALKALI HALIDE OF CALCIUM  
Otto G. Koppius, Florence, Ky., assignor of fifteen percent  
to Michael Ebert, New York, N.Y.  
Filed Jan. 27, 1967, Ser. No. 612,189

Int. Cl. H01j 19/06

U.S. CL. 313—346

4 Claims

## ABSTRACT OF THE DISCLOSURE

A secondary emission cathode structure or dynode formed from a porous matrix of tungsten or molybdenum impregnated with molten secondary emission material which is either an oxidic compound, such as tungstates, or a halide compound such as alkali halides of calcium.

This invention relates generally to secondary emission cathode structures or dynodes and methods of fabricating such structures.

Almost all metals and some insulators will emit secondary electrons when bombarded by a stream of primary electrons or ions. The number of secondary electrons emitted per primary electron depends on the velocity of the bombarding electrons and upon the nature of the material, as well as the condition of its surface. The number of secondaries liberated per primary electron may be greater than one for the velocity of the secondary electrons is lower than that of the primaries. A secondary emission element when used as an electrode in an electron tube having a collector electrode or anode for secondary electrons is known as a dynode, as distinguished from the term cathode which, when unqualified, is ordinarily an emitter of primary electrons. The terms "dynode" and "secondary emission cathode" are used interchangeably herein.

Currently, the phenomenon of secondary electron emission is used in a number of tubes of commercial significance such as photomultipliers, image converters and storage tubes. Recently the secondary emitter effect has become important in the crossfield microwave tube technology wherein a cold, secondary emission cathode is called for that can stand severe back bombardment under high power requirements. A further requirement usually stipulated is that such a cathode produce no primary electrons.

Secondary emission cathodes now in use are generally of the thin film variety of the type,  $SbCo_3$  and others. These are completely unstable under high electron bombardment and at elevated temperatures. It is well known, for example, that the alkali halides have a high secondary emission. However, if a layer of such a compound is bombarded with electrons, a decrease of the secondary emission yield usually occurs. This happens especially to layers of alkali halogenides evaporated in vacuo. The decomposition of the compound, with a consequent decrease in secondary emission yield, is one of the major problems when electron multiplication is required at high current densities.

Accordingly, it is the main object of this invention to provide a secondary emission cathode structure or dynode which produces no primary electrons and which is highly stable under heavy electron bombardment at elevated temperatures.

More specifically, it is the object of this invention to provide a dynode constituted by a porous metallic matrix within which a secondary emission compound is dispersed,

the melting point of the compound having been adjusted so that it will migrate to the surface of the matrix at a given temperature depending on the operating characteristics of the specific tube in which it is installed; this temperature being as low as  $600^{\circ}$  C. or as high as  $1100^{\circ}$  C., whereby the active secondary emitter material on the cathode surface is continuously replenished and secondary emission remains constant. Briefly stated, these objects are accomplished by:

(A) A porous structure made from either molybdenum or tungsten as the preferred base material in which the secondary electron emitter is dispersed.

(B) The porous tungsten or molybdenum matrix is impregnated with the molten secondary electron emitter.

(C) The molten secondary electron emitter can be either an oxidic compound or a halide compound.

(D) The preferred compounds for secondary electron emission at high temperatures, i.e.,  $900^{\circ}$ — $1100^{\circ}$  C., are the tungstates and molybdates of barium, strontium, calcium and magnesium. The preferred compound is barium tungstate. (The tungstates and molybdates may be considered as a mixture of two oxides, i.e., barium tungstate  $BaO \cdot WO_3$ , barium molybdate  $BaO \cdot MoO_3$ , etc.)

(E) The preferred halides are the alkali halides of calcium fluoride, barium fluoride, magnesium fluoride, and lithium fluoride. These are listed in order of preference. (Halides are binary compounds of halogen, such as chlorine, fluorine, iodine, etc., with a more electro-positive element such as sodium, potassium, iron, aluminum, etc.)

(F) The preferred alkali halide eutectic mixtures are:

LiF—NaF—CaF<sub>2</sub>

LiF—NaF—MgF<sub>2</sub>

BaF<sub>2</sub>—CaF<sub>2</sub>—LiF

LiF—CaF<sub>2</sub>—MgF<sub>2</sub>

BaF<sub>2</sub>—LiF—MgF<sub>2</sub>

Secondary emission cathodes using eutectic mixtures of these five systems have been adjusted to operate between about  $600^{\circ}$  C. to  $900^{\circ}$  C. with excellent life and high secondary yield.

For a better understanding of the invention, reference is made to the following detailed description to be read in conjunction with the accompanying drawing whose single figure is a flow chart showing the steps involved in making the cathode in accordance with the invention.

It has been found experimentally that elastic reflection of the primary electrons decreases with increasing energy such that at an energy of 20 electron-volts, 40% of the total secondary electrons consist of elastically reflected electrons, whereas this percentage drops below 10 for primary electrons with an energy of 100 electron-volts. (One electron-volt is the energy required by an electron when it is accelerated through a potential difference of one volt, i.e., 1 ev.)

Within the energy range between 100 and 2000 electron volts the slow electrons, i.e., true secondary electrons, are the larger fraction of the total secondary electron current. It is within this range of energy that most secondary emission effects are measured and made use of commercially. Further, a precedent has been established for calling all emitted electrons secondary electrons. It has been tacitly assumed that all emitted electrons are emitted by the impinging primary electrons. Although incorrect, it is useful when the aim is to find gross effects, i.e., which substances are able to emit very many or very few secondary electrons. The yield of secondary electrons is defined as the proportion,  $\delta$ , of the total emitted secondary electron current to the primary electron current. The symbol,  $\delta$ , gives the number of secondary electrons emitted by the action of one primary electron. For purposes of

this patent application only  $\delta$  values of greater than one are of interest.

The secondary electron emission at very low primary energy, i.e., 10 ev. or less, has been found to be determined by the work function of the material. Since for most practical microwave tubes, the primary energy far exceeds this value, the work function of the material plays no part in the secondary emission. In fact for most applications a high value of the work function is desirable.

The secondary electron emission at high primary electron energy, i.e., 2000 ev. or more, becomes smaller and smaller as the primary electron energy is increased and one observes more and more inelastically scattered electrons. The higher the density of the bombarded material, the greater the number of secondary electrons one observes. Some microwave tubes utilize electrons with energies in excess of 2000 ev. and for this reason the porous metal matrix within which the secondary emitting material is dispersed should be of high density, such as tungsten, in order to maximize the number of elastically scattered electrons.

The secondary electron emission yield of metals has been found to be almost completely independent of the temperature. This can be understood since the energies of the secondary electrons are large compared to the increased thermal energy contributed by heating the secondary emitter material. With secondary emitter materials involving poor electrical conducting compounds, such as NaF, BaF<sub>2</sub>, Al<sub>2</sub>O<sub>3</sub>, etc., the situation is more complicated. These materials are usually deposited as a layer over a metallic base. Under primary electron bombardment this layer will build up a charge which would make secondary emission impossible. Since the conductivity of most insulators increases with increasing temperature, then a temperature secondary electron emission dependence is observed. The new cathode which will be described later in greater detail, does not show this effect, or at least it is negligible for all practical purposes.

The secondary electron emission coefficient,  $\delta$ , for metals using primary electron bombarding energies from 0 to 1500 ev. shows a maximum value of the coefficient. The curve rises rapidly with increasing primary energy to a broad maximum and then slowly declines. The maximum can be explained by the fact that an increasing primary energy increases the number of secondary electrons generated, but the depth at which secondary electrons are released also increases and there is an increasing loss by absorption. For over thirty different metals the coefficient,  $\delta$ , has a maximum of 1.8 for platinum and a minimum value of 0.5 for lithium. For most metals the coefficient falls between 1 and 1.5. The maximum value of the coefficient,  $\delta$ , occurs for the majority of the metals at a primary electron energy between about 200-800 ev. From this data it is evident that the choice of the type of matrix base metal within which the secondary emissive material is dispersed is not determined by the  $\delta$  coefficient. Other considerations are more important such as the melting point, thermal stability, chemical activity, etc., of the matrix metal.

Secondary electron emission from metal compounds is an extremely complicated phenomena. Many compounds are not at all stable under electron bombardment. Most are electrical insulators as a consequence of which surface charge phenomena have a definite influence on the secondary emission. Technically these substances are even more important than the metals since many of the compounds give a high yield. The highest values of  $\delta$ -max. are found with simple compounds of the alkali metals, such as oxides, halides, etc. Yields are somewhat smaller from the simple compounds of the alkaline earth metals, smaller still from the oxides of aluminum, silicon, etc. A few examples are given below.

| Compound         | $\delta$ -Max. | Compound                       | $\delta$ Max. |
|------------------|----------------|--------------------------------|---------------|
| LiF              | 5.6            | BeO                            | 3.4           |
| NaF              | 5.7            | MgO                            | 4.0-2.4       |
| NaCl             | 6.8            | BaO                            | 2.3-4.8       |
| KCl              | 7.5            | Al <sub>2</sub> O <sub>3</sub> | 1.5-4.8       |
| CaF <sub>2</sub> | 3.2            | SiO <sub>2</sub>               | 2.1-2.9       |
| BaF <sub>2</sub> | 4.5            | CaO                            | 2.2           |

There are a number of complications connected with secondary electron emission from compounds. As was mentioned previously, most are insulators and the lack of conductivity causes the potential of the emitting surface to be ill defined. In a cathode in accordance with the invention, the lack of conductivity has been minimized by dispersing the emitting agent in a good conducting metal. The close proximity of the metal matrix to the secondary emission insulator permits the charge on its surface to be removed rapidly.

Further, since the melting point of the emitting agent has been adjusted to be close to the operating temperature of the cathode, the conductivity of the emitter material increases to a value that no charge remains on the surface.

The most serious limitation of the use of compounds for secondary electron emission is their lack of stability under severe electron bombardment. Such compounds initially have a high secondary yield and then under electron bombardment rapidly deteriorate. For example, an evaporated layer of sodium chloride initially has a  $\delta$  coefficient of about 5.5 at a primary electron bombardment energy of 600 ev. which then drops to less than 4.0 within about 30 minutes. The accepted explanation of this is a bit complicated. The electrons emitted from the sodium chloride layer are those with the highest energy in the crystal, i.e., those occupying the highest energy band. If one of these electrons is emitted a chlorine atom is left in the crystal. Two things could happen to the chlorine atom:

- (1) the chlorine atom could remain in the crystal lattice,
- (2) the chlorine atom could escape from the lattice.

Upon the ejection of the electron a positive charge is left behind which then must be neutralized by an electron from the base material on which the sodium chloride layer is deposited. In the first instance the positive charge on the chlorine atom is neutralized by recombination with the electron from the base. In the second case the chlorine atom has disappeared from the crystal lattice. Neutrality can be established by an electron moving from the base material into the remaining hole. The electron is now trapped and it behaves like a neutral atom. It is known as a "color center." As more and more "color centers" are formed the remaining sodium atoms form a colloidal dispersion of metal particles in the sodium chloride layer with the consequence that the secondary electron emission drops.

This is because the,  $\delta$ , coefficient is less for metallic sodium than for sodium chloride. If the sodium chloride layer is now heated to below its melting point the color centers disappear, and the secondary electron emission yield is re-established. The melting point of the secondary emission material in the cathode according to the invention has been adjusted such that this phenomena is minimized. That is, the secondary emission material is dispensed, or rejuvenated in the new cathode.

The requirements for a secondary electron emission cathode for microwave tubes are stringent. The  $\delta$  coefficient should be the order of 2 or better. The cathode must be able to withstand considerable back electron bombardment without deterioration. In the event that a primary electron source is used in the tube to supply the initial electrons, the deterioration products, if any, of the secondary electron emitter must not poison the primary emitter.

Some tubes do not require a primary source of electrons and in this event the choice of secondary electron emitter material is much broader than in the other case.

Under back electron bombardment the secondary emitter may run as cool as 600° C. or as hot as 1100° C. Moreover, in some tubes, due to a sudden change in load or a change in impedance, a given tube whose secondary emitting cathode is operating at a temperature of 600° C. may jump to 800° C. due to a change in back bombardment. The characteristics of the secondary emitter must not be permanently affected by this change in temperature.

A general requirement for most secondary electron emitters is that it must not emit primary electrons. This requirement becomes more and more difficult to satisfy as the operating temperature of the secondary emitter is increased. At the lower temperature, that is, below 700° C., secondary emissive materials that are good primary emitters at 1050° C. can be used but most of these materials have high melting points and at the lower temperatures they supply no dispenser action. For this reason they may have a good but finite life before the secondary electron emission begins to decay.

For economic reasons, most tube engineers prefer not to put auxiliary heaters in secondary emitter cathodes in order to properly activate it. Dynodes employing a porous tungsten matrix impregnated with barium calcium aluminate with a mole ratio of 4:1:1 and/or 5:3:2, require an activation at 1100° C. in high vacuum for several hours before the secondary electron emission becomes stable after the cathode temperature is lowered below 700° C.

Since this cathode is a good primary electron emitter at the activation temperature, it must be operated as a secondary emission cathode below 700° C. if primary electrons are to be avoided. At this temperature no dispenser action of the emitter material occurs and the secondary emission has a limited life. Since most microwave tubes are processed at a bake-out temperature of about 600° C., a secondary emission cathode that will activate at this temperature is desirable since in this event no auxiliary heaters are necessary. Finally, the secondary electron cathode must be stable physically, that is, its geometrical configuration must not change, also there is a preference for cathodes made from non-magnetic materials.

Porous tungsten and molybdenum have been found to be the most desirable matrix base metal. They are not magnetic and are stable geometrically under the conditions of tube operation. The preferred method of making porous tungsten and/or porous molybdenum involves Steps I through V, as described below for tungsten which includes the impregnation of the porous tungsten metal with one of the preferred secondary emissive compounds, barium tungstate.

Step I.—Tungsten powders having a mean particle size of 4.5 microns are pressed in a suitable die into bars or other suitable shapes, using a pressure of 10,000 to 30,000 p.s.i., preferably of 20,000 p.s.i. Such green bars, even without the use of a binder, have sufficient coherence and strength to be handled, and they can be readily shaped by hand tools.

Step II.—The green tungsten bars are then loaded into a high-temperature sintering furnace where the temperature is slowly raised to about 2360° C., and maintained at this level for about 20 minutes. It has been found that for 4.5 micron commercial tungsten powders pressed at 20,000 p.s.i. and sintered at 2360° C. for 20 minutes, the resultant structure has a density of 84% of theoretical. It will be appreciated that by proper adjustment of time and sintering temperature parameters, other values of theoretical density may be obtained.

Step III.—For purposes of quality control, the porous tungsten bars formed in Step II are weighed first in air and then weighed again when submerged in mercury. From these two values the percentage of theoretical density can be computed. If the percentage falls below the desired amount, the bars can be resintered until the requisite value is attained. To insure uniform skeletons, 70

the theoretical density should be held to within plus and minus 2%.

Step IV.—The porous sintered tungsten bars are then loaded into a high-temperature impregnation furnace having a hydrogen atmosphere. An amount of barium tungstate sufficient to effect complete impregnation is placed around and in contact with the bars. The furnace temperature is then slowly elevated until the barium tungstate becomes molten and starts to wet the porous tungsten skeletons. At this point, the temperature is 1650° C., the melting point of barium tungstate, which is still well below the sintering temperature of the tungsten. This temperature level is held for about 10 minutes, and as a result, all pores of the tungsten skeleton are filled with the molten barium tungstate. The furnace temperature is then quickly reduced to room temperature.

Step V.—Finally, the tungsten bars impregnated with barium tungstate are machined to the required dynode specifications to produce a secondary emission structure.

In addition to barium tungstate, the following compounds are good secondary emitters having a  $\delta$  coefficient of about 3. These are classed as high temperature melting compounds with a very poor to poor primary emission at 1050° C.

- 20 25 (1) Strontium aluminate ( $\text{SrO:Al}_2\text{O}_3$ )
- (2) Strontium, calcium aluminate ( $\text{SrO:CaO:Al}_2\text{O}_3$ )
- (3) Barium silicate ( $\text{BaO:SiO}_2$ )
- (4) Barium, calcium silicate ( $\text{BaO:CaO:SiO}_2$ )
- (5) Barium beryllate ( $\text{BaO:BeO}$ )
- (6) Barium, calcium beryllate ( $\text{BaO:CaO:BeO}$ )
- (7) Barium calcium borate ( $\text{BaO:CaO:B}_2\text{O}_3$ )
- (8) Barium, silicon aluminate ( $\text{BaO:SiO}_2\text{Al}_2\text{O}_5$ )
- (9) Barium, calcium titanate ( $\text{BaO:CaO:TiO}_2$ )
- (10) Magnesium ferrite ( $\text{MgO:Fe}_2\text{O}_3$ )
- (11) Barium titanate ( $\text{BaO:TiO}_2$ )
- (12) Barium, calcium titanate ( $\text{BaO:CaO:TiO}_2$ )
- (13) Calcium silicate ( $\text{CaO:SiO}_2$ )
- (14) Calcium titanate ( $\text{CaO:TiO}_2$ )
- (15) Barium zirconate ( $\text{BaO:ZrO}_2$ )
- (16) Calcium zirconate ( $\text{CaO:ZrO}_2$ )
- (17) Magnesium zirconate ( $\text{MgO:ZrO}_2$ )

The above compounds are exceedingly stable under electron bombardment, and work well as secondary electron emissive material when impregnated into either porous tungsten or molybdenum. Compounds like barium calcium aluminate have to be activated at 1100° C. in vacuum for a period of time in order to have a stable secondary electron emission yield at temperatures below 700° C.

The most important compounds for secondary electron emission yield at high temperatures are the tungstates and the molybdates of barium, strontium, calcium and magnesium. Of these barium tungstate is the compound preferred. It is the most stable one chemically. All of the tungstates and molybdates give no primary emission at 1050° C. provided of course the compounds are of high purity. The secondary electron emission coefficient,  $\delta$ , has a value between 2 and 3.

Porous tungsten dynodes having a theoretical density between 80-84% of pure tungsten impregnated with molten barium tungstate have been found to have thousands of hours life when run between 900° C. and 1050° C. in magnetrons under severe bombardment. The operation temperature, i.e., 900°-1050° C. is close enough to the melting point of barium tungstate that rapid diffusion of the emitter material occurs over the tungsten surface and a dispenser action maintains the emitter material on the surface. Further, the operating temperature is sufficiently high that the "color centers" are destroyed as fast as they are formed and the secondary electron emission yield holds at a high level. If the secondary emitter temperature is decreased to below about 700° C. then such a cathode has only a life of a few hundred hours before the

secondary emission drops. No dispenser action occurs at this temperature.

The highest yield of secondary electrons has been obtained from the fluorides of calcium, barium, sodium, lithium, and magnesium. These, when mixed together, form low temperature melting eutectics. Further, they have been found to wet in the molten state both porous tungsten and porous molybdenum. The impregnation of the porous metal matrix by these molten alkali halides is complete. Also and most important, the resultant impregnated metal matrix can be machined with ease by conventional machine tools. In this case the fluoride impregnant acts very much the same for machining purposes as if the porous matrix was either impregnated with molten copper or a plastic.

The preferred secondary electron emitter is calcium fluoride as it is the most stable and it has been found to have a high yield of secondary electrons. The coefficient,  $\delta$ , exceeds 3 and in a number of tests was as high as 8. The order of preference after calcium fluoride is barium fluoride, magnesium fluoride, sodium fluoride, and lithium fluoride. The,  $\delta$ , coefficient for these is about 5. The melting points of these alkali halides are listed below:

|                        | ° C. |
|------------------------|------|
| CaF <sub>2</sub> ----- | 1418 |
| BaF <sub>2</sub> ----- | 1280 |
| MgF <sub>2</sub> ----- | 1270 |
| NaF -----              | 980  |
| LiF -----              | 844  |

These secondary electron emitters can be used individually, as a combination of two compounds, as a combination of three compounds, and even as a combination of four compounds.

The following five fluoride systems of three compounds each have been found to have extraordinarily good secondary electron emission properties in that the yield is above 5 for all combinations:



The melting point of the eutectic mixtures can be changed from a low value of about 600° C. to about 1200° C. by changing the amount of each of the three compounds used to form the emitter material.

Since the melting points of the fluoride systems can be changed over a wide range it is possible to pick an optimum mixture which has a melting point sufficiently close to the operating temperature of the secondary emitter that dispenser action occurs. Further, under these condi-

tions the "color centers" formed during bombardment by the primary electrons are destroyed and the yield of secondary electrons continues at a high level. Finally, since the melting temperature of the alkali halide mixtures can be adjusted to a value close to the bake-out temperature of the tube, no further activation of the secondary emitter cathode is required.

The fluoride systems are most useful in those microwave tubes requiring no source of primary electrons. In tubes using a primary electron source it is necessary to use a very good barium getter to insure continued primary cathode activity.

While there have been shown preferred embodiments of the invention, it is to be understood that many modifications may be made therein without departing from the essential spirit of the invention as defined in the annexed claims.

What I claim is:

1. An electron tube having a dynode and means to subject said dynode to electron bombardment to an extent causing it to operate at a temperature in a range of 600° C. to 1100° C. without emission of primary electrons, said dynode comprising:

(A) a matrix formed of a porous metal selected from a class consisting of molybdenum and tungsten, and (B) a secondary emission material impregnating the pores of said matrix and having a melting point at which, in the operating range of the dynode, causes the material to migrate to the surface of the matrix, said material being selected from a class consisting of an oxidic compound and a halide compound.

2. A dynode, as set forth in claim 1, wherein said oxidic compounds are the tungstates and molybdates of barium, strontium, calcium and magnesium.

3. A dynode as set forth in claim 1, wherein said oxidic compound is barium tungstate.

4. A dynode as set forth in claim 1, wherein said halide compounds are the alkali halides of calcium fluoride, barium fluoride, magnesium fluoride, and lithium fluoride.

#### References Cited

#### UNITED STATES PATENTS

|           |        |                        |         |
|-----------|--------|------------------------|---------|
| 3,297,901 | 1/1967 | MacDonald et al. ----- | 313—346 |
| 3,118,080 | 1/1964 | Koppius -----          | 313—337 |
| 3,197,662 | 7/1965 | Schneeberger -----     | 313—104 |

JOHN W. HUCKERT, Primary Examiner

B. ESTRIN, Assistant Examiner

U.S. CL. X.R.

252—521; 313—337